



US007867675B2

(12) **United States Patent**  
**Wu et al.**

(10) **Patent No.:** **US 7,867,675 B2**  
(45) **Date of Patent:** **Jan. 11, 2011**

(54) **NITROGEN HETEROCYCЛИCS IN  
PHOTOCODUCTOR CHARGE TRANSPORT  
LAYER**

JP 10048857 A \* 2/1998  
JP 11084695 A \* 3/1999

(75) Inventors: **Jin Wu**, Webster, NY (US); **Linda L Ferrarese**, Rochester, NY (US); **Marc J Livecchi**, Rochester, NY (US); **Edward C Savage**, Webster, NY (US)

(73) Assignee: **Xerox Corporation**, Norwalk, CT (US)

(\*) Notice: Subject to any disclaimer, the term of this patent is extended or adjusted under 35 U.S.C. 154(b) by 525 days.

(21) Appl. No.: **11/961,561**

(22) Filed: **Dec. 20, 2007**

(65) **Prior Publication Data**

US 2009/0162764 A1 Jun. 25, 2009

(51) **Int. Cl.**  
**G03G 5/047** (2006.01)

(52) **U.S. Cl.** ..... **430/58.5**; 430/970

(58) **Field of Classification Search** ..... 430/58.5,  
430/58.8, 58.75, 970

See application file for complete search history.

(56) **References Cited**

U.S. PATENT DOCUMENTS

- 4,265,990 A 5/1981 Stolka et al.  
4,273,846 A \* 6/1981 Pai et al. .... 430/58.75  
4,477,547 A \* 10/1984 Yamada et al. .... 430/14  
4,587,189 A 5/1986 Hor et al.  
4,921,769 A 5/1990 Yuh et al.  
5,130,222 A \* 7/1992 Otsuka et al. .... 430/56  
5,473,064 A 12/1995 Mayo et al.  
5,482,811 A 1/1996 Keoshkerian et al.  
5,521,306 A 5/1996 Burt et al.  
6,174,635 B1 \* 1/2001 Terrell et al. .... 430/56  
6,913,863 B2 7/2005 Wu et al.  
7,037,631 B2 5/2006 Wu et al.  
2004/0063012 A1 \* 4/2004 Jubran et al. .... 430/58.6  
2004/0126685 A1 \* 7/2004 Horgan et al. .... 430/58.8  
2006/0105254 A1 5/2006 Wu et al.  
2006/0269856 A1 \* 11/2006 Wu et al. .... 430/59.4  
2006/0275681 A1 \* 12/2006 Bellino et al. .... 430/58.4  
2009/0162765 A1 6/2009 Wu et al.  
2009/0162766 A1 6/2009 Wu et al.  
2009/0162767 A1 6/2009 Wu  
2009/0162768 A1 6/2009 Wu et al.  
2009/0162769 A1 6/2009 Wu

FOREIGN PATENT DOCUMENTS

JP 02285357 A \* 11/1990

OTHER PUBLICATIONS

“National Industrial Chemicals Notification and Assessment Scheme, Full Public Report, Cyasorb UV 1164”, National Occupational Health and Safety Commission of Australia, (10-98).\*

English language machine translation of JP 10-048857 (Feb. 1998).\*

English language machine translation of JP 11-084695 (Mar. 1999).\*

English language translation of JP 02-285357 (Nov. 1990).\*

Borsenberger, Paul M. et al. Organic Photoreceptors for Imaging Systems, New York:Marcel-Dekker, Inc. (1993) pp. 289-296.\*

Jin Wu, U.S. Appl. No. 11/831,440 on Additive Containing Photogenerating Layer Photoconductors, filed Jul. 31, 2007.

Jin Wu et al., U.S. Appl. No. 11/869,258 on Imidazolium Salt Containing Charge Transport Layer Photoconductors, filed Oct. 9, 2007.

Jin Wu et al., U.S. Appl. No. 11/869,252 on Additive Containing Charge Transport Layer Photoconductors, filed Oct. 9, 2007.

Jin Wu et al., U.S. Appl. No. 11/869,231 on Additive Containing Photogenerating Layer Photoconductors, filed Oct. 9, 2007.

Liang-Bih Lin et al., U.S. Appl. No. 11/800,129 on Photoconductors, filed May 4, 2007.

Liang-Bih Lin et al., U.S. Appl. No. 11/800,108 on Photoconductors, filed May 4, 2007.

Jin Wu et al., U.S. Appl. No. 11/869,269 on Charge Trapping Releaser Containing Charge Transport Layer Photoconductors, filed Oct. 9, 2007.

Jin Wu et al., U.S. Appl. No. 11/848,428 on Photoconductors, filed Aug. 31, 2007.

Jin Wu, U.S. Appl. No. 11/848,417 on Light Stabilizer Containing Photoconductors, filed Aug. 31, 2007.

Jin Wu, U.S. Appl. No. 11/848,439 on Boron Containing Photoconductors, filed Aug. 31, 2007.

Jin Wu, U.S. Appl. No. 11/848,448 on Triazole Containing Photoconductors, filed Aug. 31, 2007.

Liang-Bih Lin et al., U.S. Appl. No. 11/848,454 on Hydroxy Benzophenone Containing Photoconductors, filed Aug. 31, 2007.

Jin Wu et al., U.S. Appl. No. 11/472,765 on Titanyl Phthalocyanine Photoconductors, filed Jun. 22, 2006.

Jin Wu et al., U.S. Appl. No. 11/472,766 on Titanyl Phthalocyanine Photoconductors, filed Jun. 22, 2006.

\* cited by examiner

Primary Examiner—Christopher RoDee

(74) Attorney, Agent, or Firm—Oliff & Berridge, PLC

(57) **ABSTRACT**

A photoconductor that includes, for example, a supporting substrate, a photogenerating layer, and at least one charge transport layer comprised of at least one charge transport component, and a nitrogen heterocyclic component such as a triazine.

**20 Claims, No Drawings**

**NITROGEN HETEROCYCLICS IN  
PHOTOCOCONDUCTOR CHARGE TRANSPORT  
LAYER**

**CROSS REFERENCE TO RELATED  
APPLICATIONS**

U.S. application Ser. No. 11/961,462, U.S. Publication No. 20090162765, filed Dec. 20, 2007, entitled Ketal Containing Photoconductors, the disclosure of which is totally incorporated herein by reference, discloses a photoconductor comprising a supporting substrate, a photogenerating layer, and at least one charge transport layer comprised of at least one charge transport component, and wherein the at least one charge transport layer contains at least one ketal.

U.S. application Ser. No. 11/961,482, U.S. Patent Publication 20090162769, filed Dec. 20, 2007, entitled Phosphine Oxide Containing Photoconductors, the disclosure of which is totally incorporated herein by reference, discloses a photoconductor comprising a supporting substrate, a photogenerating layer, and at least one charge transport layer comprised of at least one charge transport component, and wherein the at least one charge transport layer contains at least one phosphine oxide.

U.S. application Ser. No. 11/961,506, U.S. Publication No. 20090162768, filed Dec. 20, 2007, entitled Aminoketone Containing Photoconductors, the disclosure of which is totally incorporated herein by reference, discloses a photoconductor comprising a supporting substrate, a photogenerating layer, and at least one charge transport layer comprised of at least one charge transport component, and wherein the at least one charge transport layer contains at least one aminoketone.

U.S. application Ser. No. 11/961,549, U.S. Patent Publication 20090162766, filed Dec. 20, 2007, entitled Photoconductors Containing Ketal Overcoats, the disclosure of which is totally incorporated herein by reference, discloses a photoconductor comprising a supporting substrate, a photogenerating layer, and at least one charge transport layer comprised of at least one charge transport component, and an overcoat layer in contact with and contiguous to the charge transport layer, and which overcoat is comprised of a crosslinked polymeric network, an overcoat charge transport component, and at least one ketal.

U.S. application Ser. No. 11/961,566, U.S. Patent Publication 20090162767, filed Dec. 20, 2007, entitled Benzophenone Containing Photoconductors, the disclosure of which is totally incorporated herein by reference, discloses a photoconductor comprising a supporting substrate, a photogenerating layer, and at least one charge transport layer comprised of at least one charge transport component, and wherein the charge transport layer contains a benzophenone.

U.S. application Ser. No. 11/831,440, U.S. Patent Publication 20090035673, filed Jul. 31, 2007 by Jin Wu, entitled Iron Containing Hole Blocking Layer Containing Photoconductors, the disclosure of which is totally incorporated herein by reference, discloses a photoconductor comprising a substrate; an undercoat layer thereover wherein the undercoat layer comprises a metal oxide, and an iron containing compound; a photogenerating layer; and at least one charge transport layer.

U.S. application Ser. No. 11/869,258, U.S. Patent Publication 20090092912, filed Oct. 9, 2007 by Jin Wu et al., entitled Imidazolium Salt Containing Charge Transport Layer Photoconductors, the disclosure of which is totally incorporated herein by reference, discloses a photoconductor comprising a supporting substrate, a photogenerating layer, and at least one charge transport layer comprised of at least one charge trans-

port component, and where at least one charge transport layer contains at least one imidazolium salt.

U.S. application Ser. No. 11/869,252, U.S. Patent Publication No. 20090092911, filed Oct. 9, 2007 by Jin Wu et al., 5 entitled Additive Containing Charge Transport Layer Photoconductors, the disclosure of which is totally incorporated herein by reference, discloses a photoconductor comprising a supporting substrate, a photogenerating layer, and at least one charge transport layer comprised of at least one charge transport component, and an ammonium salt additive or dopant.

U.S. application Ser. No. 11/869,231, U.S. Patent Publication No. 20090092913, filed Oct. 9, 2007 by Jin Wu et al., entitled Additive Containing Photogenerating Layer Photoconductors, the disclosure of which is totally incorporated herein by reference, discloses a photoconductor comprising a supporting substrate, a photogenerating layer, and at least one charge transport layer comprised of at least one charge transport component, and wherein the photogenerating layer contains at least one of an ammonium salt and an imidazolium salt.

U.S. application Ser. No. 11/800,129, U.S. Patent Publication No. 20080274419, filed May 4, 2007 by Liang-Bih Lin et al., entitled Photoconductors, the disclosure of which is totally incorporated herein by reference, discloses a photoconductor comprising a supporting substrate, a photogenerating layer, and at least one charge transport layer comprised of at least one charge transport component, and wherein the photogenerating layer contains a bis(pyridyl)alkylene.

U.S. application Ser. No. 11/800,108, now U.S. Pat. No. 7,662,526, filed May 4, 2007 by Liang-Bih Lin et al., entitled Photoconductors, the disclosure of which is totally incorporated herein by reference, discloses a photoconductor comprising a supporting substrate, a photogenerating layer, and at least one charge transport layer comprised of at least one charge transport component, and wherein the charge transport layer contains a benzoimidazolone.

U.S. application Ser. No. 11/869,269, now U.S. Pat. No. 7,709,169, filed Oct. 9, 2007 by Jin Wu, entitled Charge Trapping Releaser Containing Charge Transport Layer Photoconductors, the disclosure of which is totally incorporated herein by reference, discloses a photoconductor comprised of a supporting substrate, a photogenerating layer, and at least one charge transport layer comprised of at least one charge transport component, and wherein the at least one charge transport layer contains at least one charge trapping releaser.

U.S. application Ser. No. 11/848,428, U.S. Patent Publication No. 20090061337, filed Aug. 31, 2007, the disclosure of which is totally incorporated herein by reference, illustrates a photoconductor comprising a supporting substrate, a photogenerating layer, and at least one charge transport layer comprised of at least one charge transport component, and wherein the photogenerating layer contains a triazine.

U.S. application Ser. No. 11/848,417, U.S. Patent Publication No. 20090061336, filed Aug. 31, 2007, the disclosure of which is totally incorporated herein by reference, illustrates a photoconductor comprising a supporting substrate, a photogenerating layer, and at least one charge transport layer comprised of at least one charge transport component, and wherein the photogenerating layer contains a light stabilizer.

U.S. application Ser. No. 11/848,439, now U.S. Pat. No. 7,670,738, filed Aug. 31, 2007, the disclosure of which is totally incorporated herein by reference, illustrates a photoconductor comprising a supporting substrate, a photogenerating layer, and at least one charge transport layer comprised of at least one charge transport component, and wherein the photogenerating layer contains a boron compound.

U.S. application No. 11/848,448, now U.S. Pat. No. 7,785,758, filed Aug. 31, 2007, the disclosure of which is totally incorporated herein by reference, illustrates a photoconductor comprising a supporting substrate, a photogenerating layer, and at least one charge transport layer comprised of at least one charge transport component, and wherein the photogenerating layer contains a triazole.

U.S. application Ser. No. 11/848,454, U.S. Patent Publication 20090061340, filed Aug. 31, 2007, the disclosure of which is totally incorporated herein by reference, illustrates a photoconductor comprising a supporting substrate, a photogenerating layer, and at least one charge transport layer comprised of at least one charge transport component, and wherein the photogenerating layer contains a hydroxyalkoxy benzophenone.

In U.S. application Ser. No. 11/472,765, now U.S. Pat. No. 7,553,593, filed Jun. 22, 2006, and U.S. application Ser. No. 11/472,766, U.S. Patent Publication No. 7,485,398, filed Jun. 22, 2006, the disclosures of which are totally incorporated herein by reference, there is disclosed, for example, photoconductors comprising a photogenerating layer and a charge transport layer, and wherein the photogenerating layer contains a titanyl phthalocyanine prepared by dissolving a Type I titanyl phthalocyanine in a solution comprising a trihaloacetic acid and an alkylene halide; adding the mixture comprising the dissolved Type I titanyl phthalocyanine to a solution comprising an alcohol and an alkylene halide thereby precipitating a Type Y titanyl phthalocyanine; and treating the Type Y titanyl phthalocyanine with a monohalobenzene.

High photosensitivity titanyl phthalocyanines are illustrated in copending U.S. application Ser. No. 10/992,500, U.S. Publication No. 20060105254, the disclosures of which are totally incorporated herein by reference, which, for example, discloses a process for the preparation of a Type V titanyl phthalocyanine, comprising providing a Type I titanyl phthalocyanine; dissolving the Type I titanyl phthalocyanine in a solution comprising a trihaloacetic acid and an alkylene halide like methylene chloride; adding the resulting mixture comprising the dissolved Type I titanyl phthalocyanine to a solution comprising an alcohol and an alkylene halide thereby precipitating a Type Y titanyl phthalocyanine; and treating the Type Y titanyl phthalocyanine with monochlorobenzene to yield a Type V titanyl phthalocyanine.

A number of the components of the above cross referenced applications, such as the supporting substrates, resin binders, antioxidants, charge transport components, photogenerating pigments like hydroxygallium phthalocyanines, and titanyl phthalocyanines, high photosensitivity titanyl phthalocyanines, such as Type V, hole blocking layer components, adhesive layers, and the like, may be selected for the photoconductor and imaging members of the present disclosure in embodiments thereof.

## BACKGROUND

This disclosure is generally directed to layered imaging members, photoreceptors, photoconductors, and the like. More specifically, the present disclosure is directed to multi-layered drum, or flexible, belt imaging members, or devices comprised of a supporting medium like a substrate, a photogenerating layer, and a charge transport layer, including at least one or a plurality of charge transport layers, and wherein at least one is, for example, from 1 to about 7, from 1 to about 3, and one, and more specifically a first charge transport layer and a second charge transport layer, and wherein the charge transport layer includes a component that results in photoconductors with, it is believed, a number of advantages, such as in

embodiments, desirable light shock reductions; the minimization or substantial elimination of undesirable ghosting on developed images, such as xerographic images, including improved ghosting at various relative humidities; excellent cyclic and stable electrical properties; acceptable imaging depletion by, for example, generating free radicals which neutralize excess charges, and dark decay characteristics; minimal charge deficient spots (CDS); and compatibility with the photogenerating and charge transport resin binders. Light shock or light fatigue of photoconductors usually causes dark bands in the resulting xerographic prints from the light exposed photoconductor area at time zero, while the photoconductors disclosed herein in embodiments minimize or avoid this disadvantage in that, for example, the light shock resistant photoconductors do not usually print undesirable dark bands even when the photoconductor is exposed to light like office light sources.

At least one in embodiments refers, for example, to one, to from 1 to about 10, to from 2 to about 7; to from 2 to about 4; to 2, and the like.

Also included within the scope of the present disclosure are methods of imaging and printing with the photoconductor devices illustrated herein. These methods generally involve the formation of an electrostatic latent image on the imaging member, followed by developing the image with a toner composition comprised, for example, of thermoplastic resin, colorant, such as pigment, charge additive, and surface additive, reference U.S. Pat. Nos. 4,560,635; 4,298,697 and 4,338,390, the disclosures of which are totally incorporated herein by reference, subsequently transferring the toner image to a suitable image receiving substrate, and permanently affixing the image thereto. In those environments wherein the photoconductor is to be used in a printing mode, the imaging method involves the same operation with the exception that exposure can be accomplished with a laser device or image bar. More specifically, the flexible photoconductor belts disclosed herein can be selected for the Xerox Corporation iGEN® machines that generate with some versions over 100 copies per minute. Processes of imaging, especially xerographic imaging and printing, including digital, and/or color printing, are thus encompassed by the present disclosure. The imaging members are in embodiments sensitive in the wavelength region of, for example, from about 400 to about 900 nanometers, and in particular from about 650 to about 850 nanometers, thus diode lasers can be selected as the light source. Moreover, the imaging members of this disclosure are useful in color xerographic applications, particularly high-speed color copying and printing processes.

## REFERENCES

There is illustrated in U.S. Pat. No. 7,037,631 a photoconductive imaging member comprised of a supporting substrate, a hole blocking layer thereover, a crosslinked photogenerating layer and a charge transport layer, and wherein the photogenerating layer is comprised of a photogenerating component, and a vinyl chloride, allyl glycidyl ether, hydroxy containing polymer.

There is illustrated in U.S. Pat. No. 6,913,863, the disclosure of which is totally incorporated herein by reference, a photoconductive imaging member comprised of a hole blocking layer, a photogenerating layer, and a charge transport layer, and wherein the hole blocking layer is comprised of a metal oxide; and a mixture of a phenolic compound and a phenolic resin wherein the phenolic compound contains at least two phenolic groups.

Layered photoresponsive imaging members have been described in numerous U.S. patents, such as U.S. Pat. No. 4,265,990 wherein there is illustrated an imaging member comprised of a photogenerating layer, and an aryl amine hole transport layer. Examples of disclosed photogenerating layer components include trigonal selenium, metal phthalocyanines, vanadyl phthalocyanines, and metal free phthalocyanines.

In U.S. Pat. No. 4,921,769, there are illustrated photoconductive imaging members with blocking layers of certain polyurethanes.

Illustrated in U.S. Pat. No. 5,521,306, the disclosure of which is totally incorporated herein by reference, is a process for the preparation of Type V hydroxygallium phthalocyanine comprising the in situ formation of an alkoxy-bridged gallium phthalocyanine dimer, hydrolyzing the dimer to hydroxygallium phthalocyanine, and subsequently converting the hydroxygallium phthalocyanine product to Type V hydroxygallium phthalocyanine.

Illustrated in U.S. Pat. No. 5,482,811, the disclosure of which is totally incorporated herein by reference, is a process for the preparation of hydroxygallium phthalocyanine photogenerating pigments which comprises hydrolyzing a gallium phthalocyanine precursor pigment by dissolving the hydroxygallium phthalocyanine in a strong acid, and then reprecipitating the resulting dissolved pigment in basic aqueous media; removing any ionic species formed by washing with water, concentrating the resulting aqueous slurry comprised of water and hydroxygallium phthalocyanine to a wet cake; removing water from said slurry by azeotropic distillation with an organic solvent, and subjecting said resulting pigment slurry to mixing with the addition of a second solvent to cause the formation of said hydroxygallium phthalocyanine polymorphs.

Also, in U.S. Pat. No. 5,473,064, the disclosure of which is totally incorporated herein by reference, there is illustrated a process for the preparation of photogenerating pigments of hydroxygallium phthalocyanine Type V essentially free of chlorine, whereby a pigment precursor Type I chlorogallium phthalocyanine is prepared by reaction of gallium chloride in a solvent, such as N-methylpyrrolidone, hydrolyzing said pigment precursor chlorogallium phthalocyanine Type I by standard methods, for example acid pasting, subsequently treating the resulting hydrolyzed pigment hydroxygallium phthalocyanine Type I with a solvent, such as N,N-dimethylformamide, present in an amount of from about 1 volume part to about 50 volume parts, and preferably about 15 volume parts for each weight part of pigment hydroxygallium phthalocyanine that is used by, for example, ball milling the Type I hydroxygallium phthalocyanine pigment in the presence of spherical glass beads, approximately 1 millimeter to 5 millimeters in diameter, at room temperature, about 25° C., for a period of from about 12 hours to about 1 week, and preferably about 24 hours.

In U.S. Pat. No. 4,587,189, the disclosure of which is totally incorporated herein by reference, there is illustrated a layered imaging member with, for example, a perylene, pigment photogenerating component and an aryl amine component, such as N,N'-diphenyl-N,N'-bis(3-methylphenyl)-1,1'-biphenyl-4,4'-diamine dispersed in a polycarbonate binder as a hole transport layer.

Kanemitsu and Funada (*J. Phys. D: Appl. Phys.* 24, 1991, 1409-1415) have apparently suggested that light-induced fatigue of the photoconductor is a consequence of the build-up of the negative charges caused by electron trapping in the photogenerating layer and the positive charges caused by hole trapping at the photogenerating layer charge transport layer

interface. The photoconductors illustrated herein in embodiments, and with an additive, such as a triazine, and those additives illustrated in the appropriate copending applications filed concurrently herewith, in the charge transport layer results in reduced light shock characteristics as compared to a similar photoconductor with no charge transport layer (CTL) additive as the additive is believed to absorb the UV portion of the white light and generate active species such as free radicals that can interact with or neutralize those light (usually visible light) generated charges within the photoconductor.

The appropriate components, such as the supporting substrates, the photogenerating layer components, the charge transport layer components, and the like of the above-recited patents, may be selected for the photoconductors of the present disclosure in embodiments thereof.

## SUMMARY

Disclosed are photoconductors that contain a dopant or additive in the charge transport layer thereby permitting such photoconductors to exhibit minimal light shock characteristics.

Further, disclosed are photoconductors comprised of suitable additive containing charge transport layers, and where in embodiments the photogenerating layer further contains a photogenerating pigment or pigments, such as a high photosensitivity titanyl phthalocyanine.

Additionally, disclosed are flexible belt imaging members containing optional hole blocking layers comprised of, for example, amino silanes, metal oxides, phenolic resins, and optional phenolic compounds, and which phenolic compounds contain at least two, and more specifically, two to ten phenol groups or phenolic resins with, for example, a weight average molecular weight ranging from about 500 to about 3,000, permitting, for example, a hole blocking layer with excellent efficient electron transport which usually results in a desirable photoconductor low residual potential  $V_{low}$ .

The photoconductors illustrated herein may in embodiments have excellent wear resistance, extended lifetimes, elimination or minimization of imaging member scratches on the surface layer or layers of the member, and which scratches can result in undesirable print failures where, for example, the scratches are visible on the final prints generated. Additionally, in embodiments the imaging members disclosed herein possess high sensitivity; low acceptable image ghosting characteristics; low background and/or minimal charge deficient spots (CDS); and desirable toner cleanability. At least one in embodiments refers, for example, to one, to from 1 to about 10, to from 2 to about 7; to from 2 to about 4, to two, and the like.

## EMBODIMENTS

Aspects of the present disclosure relate to a photoconductor comprising a supporting medium, a photogenerating layer comprised of at least one photogenerating pigment, and an optional binder component, and at least one charge transport layer comprised of at least one charge transport component and a nitrogen heterocyclic component, such as a triazine; and a flexible photoconductor which includes a hole blocking layer and an adhesive layer where the adhesive layer is situated between the hole blocking layer and the photogenerating layer, and the hole blocking layer is situated between the substrate and the adhesive layer; a photoconductor comprising a supporting substrate, a photogenerating layer, and at least one charge transport layer comprised of at least one charge transport component, and a triazine; a photoconductor

comprised in sequence of a supporting substrate, a photogenerating layer comprised of at least one photogenerating pigment, and a nitrogen heterocyclic compound containing charge transport layer; and a photoconductor comprising a supporting substrate, a photogenerating layer, and a hole transport layer, wherein the hole transport layer includes at least one of the following additives, wherein n of the  $n\text{-OC}_8\text{H}_{17}$  represents normal (linear) and n' represents the number of repeating segments of from about 3 to about 10



-continued





20 Examples of charge transport layer additives present in various suitable amounts, such as from about 0.01 to about 25, about 0.05 to about 10, about 0.1 to about 5, 0.2 to about 2 weight percent based on the weight percentage of the charge transport layer components include nitrogen heterocyclic compounds like triazines.

Specific triazine examples include 2,4-bis(2,4-dimethylphenyl)-6-(2-hydroxy-4-n-octyl-oxyphenyl)-1,3,5-triazine (CYASORB® UV-1164 from CYTEC), 2,4,6-tris[di(2-pyridyl)amino]-1,3,5-triazine, 2,4,6-tris(carbazolyl)-1,3,5-triazine, 2,4,6-tris[phenyl(2-naphthanyl)amino]-1,3,5-triazine, 2,4,6-tris[phenyl(1-naphthanyl)amino]-1,3,5-triazine, 2,4,6-tris{4-[di(2-pyridyl)amino]phenyl}-1,3,5-triazine, 1,3,5-triazine, 2,4,6-tri(4-pyridyl)-1,3,5-triazine, 2,4,6-tri(2-pyridyl)-1,3,5-triazine, 2,4,6-tris[bis(methoxymethyl)amino]-1,3,5-triazine, 2,4-diamino-6-[2-(2-undecyl-1-imidazolyl)ethyl]-1,3,5-triazine, 3,4-dihydro-4-oxo-1,2,3-benzotriazine, 5,6-diphenyl-3-(2-pyridyl)-1,2,4-triazine, 40 3-amino-5,6-dimethyl-1,2,4-triazine, respectively, represented by the following formulas/structures



11



12





Other triazine examples include polymers with morpholine-2,4,6-trichloro-1,3,5-triazine, 1,6-hexanediamine, N,N'-bis(2,2,6,6-tetramethyl-4-piperidinyl)- (CYASORB® UV-3529,  $M_w \sim 1,700$  and  $n \sim 3$ ,  $T_g \sim 88^\circ C.$ ) and poly[(6-morpholino-s-triazine-2,4-diyl)[2,2,6,6-tetramethyl-4-piperidinyl]imino]-hexamethylene [(2,2,6,6-tetramethyl-4-piperidinyl)imino]] (CYASORB® UV-3346,  $M_w \sim 1,600$  and  $n \sim 3$ ), respectively, represented by the following formulas/structures



wherein  $n$  represents the number of repeating segments, and is, for example, a number of from about 1 to about 100, from about 2 to about 30, or from about 3 to about 10.

The thickness of the photoconductor substrate layer depends on many factors, including economical considerations, electrical characteristics, adequate flexibility, availability and cost of the specific components for each layer, and the like, thus this layer may be of substantial thickness, for example about 3,000 microns, such as from about 1,000 to about 2,000 microns, from about 500 to about 1,000 microns, or from about 300 to about 700 microns, ("about" throughout includes all values in between the values recited) or of a

minimum thickness. In embodiments, the thickness of this layer is from about 75 microns to about 300 microns, or from about 100 to about 150 microns.

The photoconductor substrate may be opaque or substantially transparent, and may comprise any suitable material having the required mechanical properties. Accordingly, the substrate may comprise a layer of an electrically nonconductive or conductive material such as an inorganic or an organic composition. As electrically nonconducting materials, there 10 may be employed various resins known for this purpose including polyesters, polycarbonates, polyamides, polyurethanes, and the like, which are flexible as thin webs. An electrically conducting substrate may be any suitable metal of, for example, aluminum, nickel, steel, copper, and the like, 15 or a polymeric material, as described above, filled with an electrically conducting substance, such as carbon, metallic powder, and the like, or an organic electrically conducting material. The electrically insulating or conductive substrate may be in the form of an endless flexible belt, a web, a rigid 20 cylinder, a sheet, and the like. The thickness of the substrate layer depends on numerous factors, including strength desired and economical considerations. For a drum, this layer may be of substantial thickness of, for example, up to many centimeters or of a minimum thickness of less than a millimeter. Similarly, a flexible belt may be of a substantial thickness of, for example, about 250 micrometers, or of a minimum thickness of less than about 50 micrometers, provided 25 there are no adverse effects on the final electrophotographic device.

30 In embodiments where the substrate layer is not conductive, the surface thereof may be rendered electrically conductive by an electrically conductive coating. The conductive coating may vary in thickness over substantially wide ranges depending upon the optical transparency, degree of flexibility desired, and economic factors.

Illustrative examples of substrates are as illustrated herein, and more specifically, supporting substrate layers selected for the photoconductors of the present disclosure, and which substrates can be opaque or substantially transparent comprise a layer of insulating material including inorganic or organic polymeric materials, such as MYLAR® a commercially available polymer, MYLAR® containing titanium, a layer of an organic or inorganic material having a semiconductive surface layer, such as indium tin oxide, or aluminum 40 arranged thereon, or a conductive material inclusive of aluminum, chromium, nickel, brass, or the like. The substrate may be flexible, seamless, or rigid, and may have a number of many different configurations, such as for example, a plate, a cylindrical drum, a scroll, an endless flexible belt, and the 45 like. In embodiments, the substrate is in the form of a seamless flexible belt. In some situations, it may be desirable to coat on the back of the substrate, particularly when the substrate is a flexible organic polymeric material, an anticurl layer, such as for example polycarbonate materials commercially available as MAKROLON®.

Generally, the photogenerating layer can contain known photogenerating pigments, such as metal phthalocyanines, metal free phthalocyanines, alkylhydroxyl gallium phthalocyanines, hydroxylgallium phthalocyanines, chlorogallium 50 phthalocyanines, perylenes, especially bis(benzimidazo) perylene, titanyl phthalocyanines, and the like, and more specifically, vanadyl phthalocyanines, Type V hydroxylgallium phthalocyanines, high sensitivity titanyl phthalocyanines, and inorganic components such as selenium, selenium alloys, and trigonal selenium. The photogenerating pigment 55 can be dispersed in a resin binder similar to the resin binders selected for the charge transport layer, or alternatively no

## 15

resin binder need be present. Generally, the thickness of the photogenerating layer depends on a number of factors, including the thicknesses of the other layers and the amount of photogenerating material contained in the photogenerating layer. Accordingly, this layer can be of a thickness of, for example, from about 0.05 micron to about 10 microns, and more specifically, from about 0.25 micron to about 2 microns when, for example, the photogenerating compositions are present in an amount of from about 30 to about 75 percent by volume. The maximum thickness of this layer in embodiments is dependent primarily upon factors, such as photosensitivity, electrical properties, and mechanical considerations.

The photogenerating composition or pigment can be present in a resinous binder composition in various amounts inclusive of up to 100 percent by weight. Generally, however, from about 5 percent by volume to about 95 percent by volume of the photogenerating pigment is dispersed in about 95 percent by volume to about 5 percent by volume of the resinous binder, or from about 20 percent by volume to about 30 percent by volume of the photogenerating pigment is dispersed in about 70 percent by volume to about 80 percent by volume of the resinous binder composition. In one embodiment, about 90 percent by volume of the photogenerating pigment is dispersed in about 10 percent by volume of the resinous binder composition, and which resin may be selected from a number of known polymers, such as poly(vinyl butyral), poly(vinyl carbazole), polyesters, polycarbonates, poly(vinyl chloride), polyacrylates and methacrylates, copolymers of vinyl chloride and vinyl acetate, phenolic resins, polyurethanes, poly(vinyl alcohol), polyacrylonitrile, polystyrene, and the like. It is desirable to select a coating solvent that does not substantially disturb or adversely affect the other previously coated layers of the device. Examples of coating solvents for the photogenerating layer are ketones, alcohols, aromatic hydrocarbons, halogenated aliphatic hydrocarbons, ethers, amines, amides, esters, and the like. Specific solvent examples are cyclohexanone, acetone, methyl ethyl ketone, methanol, ethanol, butanol, amyl alcohol, toluene, xylene, chlorobenzene, carbon tetrachloride, chloroform, methylene chloride, trichloroethylene, tetrahydrofuran, dioxane, diethyl ether, dimethyl formamide, dimethyl acetamide, butyl acetate, ethyl acetate, methoxyethyl acetate, and the like.

The photogenerating layer may comprise amorphous films of selenium and alloys of selenium and arsenic, tellurium, germanium, and the like, hydrogenated amorphous silicon and compounds of silicon and germanium, carbon, oxygen, nitrogen, and the like fabricated by vacuum evaporation or deposition. The photogenerating layers may also comprise inorganic pigments of crystalline selenium and its alloys; Groups II to VI compounds; and organic pigments such as quinacridones, polycyclic pigments such as dibromoanthanthrone pigments, perylene and perinone diamines, polynuclear aromatic quinones, azo pigments including bis-, tris- and tetrakis-azos, and the like dispersed in a film forming polymeric binder and fabricated by solvent coating techniques.

In embodiments, examples of polymeric binder materials that can be selected as the matrix for the photogenerating layer are illustrated in U.S. Pat. No. 3,121,006, the disclosure of which is totally incorporated herein by reference. Examples of binders are thermoplastic and thermosetting resins, such as polycarbonates, polyesters, polyamides, polyurethanes, polystyrenes, polyarylethers, polyarylsulfones, polybutadienes, polysulfones, polyethersulfones, polyethylenes, polypropylenes, polyimides, polymethylpentenes, poly(phenylene sulfides), poly(vinyl acetate), polysiloxanes,

## 16

polyacrylates, polyvinyl acetals, polyamides, polyimides, amino resins, phenylene oxide resins, terephthalic acid resins, phenoxy resins, epoxy resins, phenolic resins, polystyrene, and acrylonitrile copolymers, poly(vinyl chloride), vinyl chloride and vinyl acetate copolymers, acrylate copolymers, alkyd resins, cellulosic film formers, poly(amideimide), styrenebutadiene copolymers, vinylidene chloride-vinyl chloride copolymers, vinyl acetate-vinylidene chloride copolymers, styrene-alkyd resins, poly(vinyl carbazole), and the like. These polymers may be block, random, or alternating copolymers.

Various suitable and conventional known processes may be used to mix, and thereafter apply the photogenerating layer coating mixture like spraying, dip coating, roll coating, wire wound rod coating, vacuum sublimation, and the like. For some applications, the photogenerating layer may be fabricated in a dot or line pattern. Removal of the solvent of a solvent-coated layer may be effected by any known conventional techniques such as oven drying, infrared radiation drying, air drying, and the like.

The final dry thickness of the photogenerating layer is as illustrated herein, and can be, for example, from about 0.01 to about 30 microns after being dried at, for example, about 40° C. to about 150° C. for about 15 to about 90 minutes. More specifically, a photogenerating layer of a thickness, for example, of from about 0.1 to about 30, or from about 0.5 to about 10 microns can be applied to or deposited on the substrate, on other surfaces in between the substrate and the charge transport layer, and the like. A charge blocking layer or hole blocking layer may optionally be applied to the electrically conductive surface prior to the application of a photogenerating layer. When desired, an adhesive layer may be included between the charge blocking or hole blocking layer or interfacial layer and the photogenerating layer. Usually, the photogenerating layer is applied onto the blocking layer, and a charge transport layer or plurality of charge transport layers are formed on the photogenerating layer. This structure may have the photogenerating layer on top of or below the charge transport layer.

In embodiments, a suitable known adhesive layer can be included in the photoconductor. Typical adhesive layer materials include, for example, polyesters, polyurethanes, and the like. The adhesive layer thickness can vary and in embodiments is, for example, from about 0.05 micrometer (500 Angstroms) to about 0.3 micrometer (3,000 Angstroms). The adhesive layer can be deposited on the hole blocking layer by spraying, dip coating, roll coating, wire wound rod coating, gravure coating, Bird applicator coating, and the like. Drying of the deposited coating may be effected by, for example, oven drying, infrared radiation drying, air drying, and the like.

As optional adhesive layers usually in contact with or situated between the hole blocking layer and the photogenerating layer, there can be selected various known substances inclusive of copolymers, polyamides, poly(vinyl butyral), poly(vinyl alcohol), polyurethane, and polyacrylonitrile. This layer is, for example, of a thickness of from about 0.001 micron to about 1 micron, or from about 0.1 to about 0.5 micron. Optionally, this layer may contain effective suitable amounts, for example from about 1 to about 10 weight percent, of conductive and nonconductive particles, such as zinc oxide, titanium dioxide, silicon nitride, carbon black, and the like, to provide, for example, in embodiments of the present disclosure further desirable electrical and optical properties.

The optional hole blocking or undercoat layers for the imaging members of the present disclosure can contain a number of components including known hole blocking com-

ponents, such as amino silanes, doped metal oxides, a metal oxide like titanium, chromium, zinc, tin and the like; a mixture of phenolic compounds and a phenolic resin or a mixture of two phenolic resins, and optionally a dopant such as  $\text{SiO}_2$ . The phenolic compounds usually contain at least two phenol groups, such as bisphenol A (4,4'-isopropylidenediphenol), E (4,4'-ethyldenebisphenol), F (bis(4-hydroxyphenyl)methane), M (4,4'-(1,3-phenylenediisopropylidene)bisphenol), P (4,4'-(1,4-phenylene diisopropylidene)bisphenol), S (4,4'-sulfonyldiphenol), and Z (4,4'-cyclohexylidenebisphenol); hexafluorobisphenol A (4,4'-(hexafluoro isopropylidene) diphenol), resorcinol, hydroxyquinone, catechin, and the like.

The hole blocking layer can be, for example, comprised of from about 20 weight percent to about 80 weight percent, and more specifically, from about 55 weight percent to about 65 weight percent of a suitable component like a metal oxide, such as  $\text{TiO}_2$ , from about 20 weight percent to about 70 weight percent, and more specifically, from about 25 weight percent to about 50 weight percent of a phenolic resin; from about 2 weight percent to about 20 weight percent, and, more specifically, from about 5 weight percent to about 15 weight percent of a phenolic compound preferably containing at least two phenolic groups, such as bisphenol S, and from about 2 weight percent to about 15 weight percent, and more specifically, from about 4 weight percent to about 10 weight percent of a plywood suppression dopant, such as  $\text{SiO}_2$ . The hole blocking layer coating dispersion can, for example, be prepared as follows. The metal oxide/phenolic resin dispersion is first prepared by ball milling or dynomilling until the median particle size of the metal oxide in the dispersion is less than about 10 nanometers, for example from about 5 to about 9. To the above dispersion are added a phenolic compound and dopant followed by mixing. The hole blocking layer coating dispersion can be applied by dip coating or web coating, and the layer can be thermally cured after coating. The hole blocking layer resulting is, for example, of a thickness of from about 0.01 micron to about 30 microns, and more specifically, from about 0.1 micron to about 8 microns. Examples of phenolic resins include formaldehyde polymers with phenol, p-tert-butylphenol, cresol, such as VARCUM<sup>TM</sup> 29159 and 29101 (available from OxyChem Company), and DURITE<sup>TM</sup> 97 (available from Borden Chemical); formaldehyde polymers with ammonia, cresol and phenol, such as VARCUM<sup>TM</sup> 29112 (available from OxyChem Company); formaldehyde polymers with 4,4'-(1-methylethylidene)bisphenol, such as VARCUM<sup>TM</sup> 29108 and 29116 (available from OxyChem Company); formaldehyde polymers with cresol and phenol, such as VARCUM<sup>TM</sup> 29457 (available from OxyChem Company), DURITE<sup>TM</sup> SD-423A, SD-422A (available from Borden Chemical); or formaldehyde polymers with phenol and p-tert-butylphenol, such as DURITE<sup>TM</sup> ESD 556C (available from Borden Chemical).

The optional hole blocking layer may be applied to the substrate. Any suitable and conventional blocking layer capable of forming an electronic barrier to holes between the adjacent photoconductive layer (or electrophotographic imaging layer) and the underlying conductive surface of substrate may be selected.

A number of charge transport compounds can be included in the charge transport layer, which layer generally is of a thickness of from about 5 microns to about 75 microns, and more specifically, of a thickness of from about 10 microns to about 40 microns. Examples of charge transport components are aryl amines of the following formulas/structures



20 wherein X is a suitable hydrocarbon like alkyl, alkoxy, aryl, and derivatives thereof; a halogen, or mixtures thereof, and especially those substituents selected from the group consisting of Cl and  $\text{CH}_3$ ; and molecules of the following formulas



wherein X, Y and Z are independently alkyl, alkoxy, aryl, a  
45 halogen, or mixtures thereof, and wherein at least one of Y  
and Z are present.

Alkyl and alkoxy contain, for example, from 1 to about 25 carbon atoms, and more specifically, from 1 to about 12 carbon atoms, such as methyl, ethyl, propyl, butyl, pentyl, and 50 the corresponding alkoxides. Aryl can contain from 6 to about 36 carbon atoms, such as phenyl, and the like. Halogen includes chloride, bromide, iodide, and fluoride. Substituted alkyls, alkoxy, and aryls can also be selected in embodiments.

bis(4-butylphenyl)-N,N'-bis-(2,5-dimethylphenyl)-[p-terphenyl]-4,4'-diamine, N,N'-diphenyl-N,N'-bis(3-chlorophenyl)-[p-terphenyl]-4,4"-diamine, and the like. Other known charge transport layer molecules can be selected, reference for example, U.S. Pat. Nos. 4,921,773 and 4,464,450, the disclosures of which are totally incorporated herein by reference.

Examples of the binder materials selected for the charge transport layers include components, such as those described in U.S. Pat. No. 3,121,006, the disclosure of which is totally incorporated herein by reference. Specific examples of polymer binder materials include polycarbonates, polyarylates, acrylate polymers, vinyl polymers, cellulose polymers, polyesters, polysiloxanes, polyamides, polyurethanes, poly(cycloolefins), epoxies, and random or alternating copolymers thereof; and more specifically, polycarbonates such as poly(4,4'-isopropylidene-diphenylene) carbonate (also referred to as bisphenol-A-polycarbonate), poly(4,4'-cyclohexylidene-diphenylene) carbonate (also referred to as bisphenol-Z-polycarbonate), poly(4,4'-isopropylidene-3,3'-dimethyl-diphenyl) carbonate (also referred to as bisphenol-C-polycarbonate), and the like. In embodiments, electrically inactive binders are comprised of polycarbonate resins with a molecular weight of from about 20,000 to about 100,000, or with a molecular weight M, of from about 50,000 to about 100,000. Generally, the transport layer contains from about 10 to about 75 percent by weight of the charge transport material, and more specifically, from about 35 percent to about 50 percent of this material.

The charge transport layer or layers, and more specifically, a first charge transport in contact with the photogenerating layer, and thereover a top or second charge transport overcoating layer may comprise charge transporting small molecules dissolved or molecularly dispersed in a film forming electrically inert polymer such as a polycarbonate. In embodiments, "dissolved" refers, for example, to forming a solution in which the small molecule is dissolved in the polymer to form a homogeneous phase; and "molecularly dispersed in embodiments" refers, for example, to charge transporting molecules dispersed in the polymer, the small molecules being dispersed in the polymer on a molecular scale. Various charge transporting or electrically active small molecules may be selected for the charge transport layer or layers. In embodiments, charge transport refers, for example, to charge transporting molecules as a monomer that allows the free charge generated in the photogenerating layer to be transported across the transport layer.

Examples of hole transporting molecules present, for example, in an amount of from about 50 to about 75 weight percent, include, for example, pyrazolines such as 1-phenyl-3-(4'-diethylamino styryl)-5-(4"-diethylamino phenyl)pyrazoline; aryl amines such as N,N'-diphenyl-N,N'-bis(3-methylphenyl)-(1,1'-biphenyl)-4,4'-diamine, N,N'-bis(4-butylphenyl)-N,N'-di-p-tolyl-[p-terphenyl]-4,4"-diamine, N,N'-bis(4-butylphenyl)-N,N'-di-m-tolyl-[p-terphenyl]-4,4"-diamine, N,N'-bis(4-butylphenyl)-N,N'-di-o-tolyl-[p-terphenyl]-4,4"-diamine, N,N'-bis(4-butylphenyl)-N,N'-bis(4-isopropylphenyl)-[p-terphenyl]-4,4"-diamine, N,N'-bis(4-butylphenyl)-N,N'-bis(2-ethyl-6-methylphenyl)-[p-terphenyl]-4,4"-diamine, N,N'-bis(4-butylphenyl)-N,N'-bis(2,5-dimethylphenyl)-[p-terphenyl]-4,4"-diamine, and N,N'-diphenyl-N,N'-bis(3-chlorophenyl)-[p-terphenyl]-4,4"-diamine; hydrazones such as N-phenyl-N-methyl-3-(9-ethyl)carbazydyl hydrazone and 4-diethyl amino benzaldehyde-1,2-diphenyl hydrazone; and oxadiazoles such as 2,5-bis(4-N,N'-diethylaminophenyl)-1,2,4-oxadiazole, stilbenes, and the like. However, in embodiments to minimize or avoid cycle-up

in equipment, such as printers, with high throughput, the charge transport layer should be substantially free (less than about two percent) of di or triamino-triphenyl methane. A small molecule charge transporting compound that permits injection of holes into the photogenerating layer with high efficiency and transports them across the charge transport layer with short transit times includes N,N'-diphenyl-N,N'-bis(3-methylphenyl)-(1,1'-biphenyl)-4,4'-diamine, N,N'-bis(4-butylphenyl)-N,N'-di-p-tolyl-[p-terphenyl]-4,4"-diamine, 10 N,N'-bis(4-butylphenyl)-N,N'-di-m-tolyl-[p-terphenyl]-4,4"-diamine, N,N'-bis(4-butylphenyl)-N,N'-di-o-tolyl-[p-terphenyl]-4,4"-diamine, N,N'-bis(4-butylphenyl)-N,N'-bis(4-isopropylphenyl)-[p-terphenyl]-4,4"-diamine, N,N'-bis(4-butylphenyl)-N,N'-bis(2-ethyl-6-methylphenyl)-[p-terphenyl]-4,4"-diamine, N,N'-bis(4-butylphenyl)-N,N'-bis(2,5-dimethylphenyl)-[p-terphenyl]-4,4"-diamine, and N,N'-diphenyl-N,N'-bis(3-chlorophenyl)-[p-terphenyl]-4,4"-diamine, or mixtures thereof. If desired, the charge transport material in the charge transport layer may comprise a polymeric charge transport material or a combination of a small molecule charge transport material and a polymeric charge transport material.

Examples of components or materials optionally incorporated into the charge transport layers or at least one charge transport layer to, for example, enable improved lateral charge migration (LCM) resistance include hindered phenolic antioxidants, such as tetrakis methylene(3,5-di-tert-butyl-4-hydroxy hydrocinnamate) methane (IRGANOX™ 1010, available from Ciba Specialty Chemical), butylated hydroxytoluene (BHT), and other hindered phenolic antioxidants including SUMILIZER™ BHT-R, MDP-S, BBM-S, WX-R, NR, BP-76, BP-101, GA-80, GM and GS (available from Sumitomo Chemical Co., Ltd.), IRGANOX™ 1035, 1076, 1098, 1135, 1141, 1222, 1330, 1425WL, 1520L, 245, 30 255, 3114, 3790, 5057 and 565 (available from Ciba Specialties Chemicals), and ADEKA STAB™ AO-20, AO-30, AO-40, AO-50, AO-60, AO-70, AO-80 and AO-330 (available from Asahi Denka Co., Ltd.); hindered amine antioxidants such as SANOL™ LS-2626, LS-765, LS-770 and LS-744 35 (available from SNKYO CO., Ltd.), TINUVINT™ 144 and 622LD (available from Ciba Specialties Chemicals), MARK™ LA57, LA67, LA62, LA68 and LA63 (available from Asahi Denka Co., Ltd.), and SUMILIZER™ PS (available from Sumitomo Chemical Co., Ltd.); thioether antioxidants such as SUMILIZER™ TP-D (available from Sumitomo Chemical Co., Ltd.); phosphite antioxidants such as MARK™ 2112, PEP-8, PEP-24G, PEP-36, 329K and HP-10 (available from Asahi Denka Co., Ltd.); other molecules such as 40 bis(4-diethylamino-2-methylphenyl)phenylmethane (BDETPM), bis-[2-methyl-4-(N-2-hydroxyethyl-N-ethylaminophenyl)]-phenylmethane (DHTPM), and the like. The weight percent of the antioxidant in at least one of the charge transport layers is from about 0 to about 20, from about 1 to about 10, or from about 3 to about 8 weight percent.

55 A number of processes may be used to mix, and thereafter apply the charge transport layer or layers coating mixture to the photogenerating layer. Typical application techniques include spraying, dip coating, roll coating, wire wound rod coating, and the like. Drying of the charge transport deposited coating may be effected by any suitable conventional technique such as oven drying, infrared radiation drying, air drying, and the like.

60 The thickness of each of the charge transport layers in embodiments is from about 10 to about 70 micrometers, but thicknesses outside this range may in embodiments also be selected. The charge transport layer should be an insulator to the extent that an electrostatic charge placed on the hole

transport layer is not conducted in the absence of illumination at a rate sufficient to prevent formation and retention of an electrostatic latent image thereon. In general, the ratio of the thickness of the charge transport layer to the photogenerating layer can be from about 2:1 to 200:1, and in some instances 400:1. The charge transport layer is substantially nonabsorbing to visible light or radiation in the region of intended use, but is electrically "active" in that it allows the injection of photogenerated holes from the photoconductive layer, or photogenerating layer, and allows these holes to be transported through itself to selectively discharge a surface charge on the surface of the active layer. Typical application techniques include spraying, dip coating, roll coating, wire wound rod coating, and the like. Drying of the deposited coating may be effected by any suitable conventional technique, such as oven drying, infrared radiation drying, air drying, and the like. An optional overcoat layer may be applied over the charge transport layer to provide abrasion protection.

Aspects of the present disclosure relate to a photoconductive imaging member with a photogenerating layer of a thickness of from about 0.1 to about 10 microns, and at least one transport layer each of a thickness of from about 5 to about 100 microns; a photoconductor where the transport layer is of a thickness of from about 40 to about 75 microns; a member wherein the photogenerating layer contains a photogenerating pigment present in an amount of from about 5 to about 95 weight percent; a member wherein the thickness of the photogenerating layer is from about 0.1 to about 8 microns; a member wherein the photogenerating layer contains a polymer binder; a member wherein the binder is present in an amount of from about 50 to about 90 percent by weight, and wherein the total of all layer components is about 100 percent; a member wherein the photogenerating component is a titanyl phthalocyanine or a hydroxygallium phthalocyanine that absorbs light of a wavelength of from about 370 to about 950 nanometers; an imaging member wherein the supporting substrate is comprised of a conductive substrate comprised of a metal; an imaging member wherein the conductive substrate is aluminum, aluminized polyethylene terephthalate, or titanized polyethylene terephthalate; an imaging member wherein the photogenerating resinous binder is selected from the group consisting of polyesters, polyvinyl butyrls, polycarbonates, polystyrene-b-polyvinyl pyridine, and polyvinyl formals; an imaging member wherein the photogenerating pigment is a metal free phthalocyanine; an imaging member wherein the charge transport layers comprises



wherein X is selected from the group consisting of alkyl, alkoxy, aryl, and halogen; an imaging member wherein alkyl and alkoxy contains from about 1 to about 12 carbon atoms; an imaging member wherein alkyl contains from about 1 to about 5 carbon atoms; an imaging member wherein alkyl is methyl; an imaging member wherein each of, or at least one of the charge transport layers comprises



wherein X and Y are independently alkyl, alkoxy, aryl, a halogen, or mixtures thereof; an imaging member wherein alkyl and alkoxy contains from about 1 to about 12 carbon atoms; an imaging member wherein alkyl contains from about 1 to about 5 carbon atoms, and wherein the resinous binder is selected from the group consisting of polycarbonates and polystyrene; an imaging member wherein the photogenerating pigment present in the photogenerating layer is comprised of chlorogallium phthalocyanine, or Type V hydroxygallium phthalocyanine prepared by hydrolyzing a gallium phthalocyanine precursor by dissolving the hydroxygallium phthalocyanine in a strong acid, and then reprecipitating the resulting dissolved precursor in a basic aqueous media; removing any ionic species formed by washing with water; concentrating the resulting aqueous slurry comprised of water and hydroxygallium phthalocyanine to a wet cake; removing water from the wet cake by drying; and subjecting the resulting dry pigment to mixing with the addition of a second solvent to cause the formation of the hydroxygallium phthalocyanine; an imaging member wherein the Type V hydroxygallium phthalocyanine has major peaks, as measured with an X-ray diffractometer, at Bragg angles (2 theta +/- 0.2 degrees) 7.4, 9.8, 12.4, 16.2, 17.6, 18.4, 21.9, 23.9, 25.0, 28.1 degrees, and the highest peak at 7.4 degrees; a method of imaging which comprises generating an electrostatic latent image on an imaging member developing the latent image, and transferring the developed electrostatic image to a suitable substrate; a method of imaging wherein the imaging member is exposed to light of a wavelength of from about 370 to about 950 nanometers; a photoconductive member wherein the photogenerating layer is situated between the substrate and the charge transport; a member wherein the photogenerating layer is of a thickness of from about 0.1 to about 50 microns; a member wherein the photogenerating pigment is dispersed in from about 1 weight percent to about 80 weight percent of a polymer binder; a member wherein the binder is present in an amount of from about 50 to about 90 percent by weight, and wherein the total of the layer components is about 100 percent; an imaging member wherein the photogenerating component is Type V hydroxygallium phthalocyanine, Type V titanyl phthalocyanine or chlorogallium phthalocyanine, and the charge transport layer contains a hole transport of N,N'-diphenyl-N,N-bis(3-methylphenyl)-1,1'-biphenyl-4,4'-diamine, N,N'-bis(4-butylphenyl)-N,N'-di-p-tolyl-[p-terphenyl]-4,4"-diamine, N,N'-bis(4-butylphenyl)-N,N'-di-m-tolyl-[p-terphenyl]-4,4"-diamine, N,N'-bis(4-butylphenyl)-N,N'-di-o-tolyl-[p-terphenyl]-4,4"-diamine, N,N'-bis(4-butylphenyl)-N,N'-bis-(4-isopropylphenyl)-[p-terphenyl]-4,4"-diamine, N,N'-bis(4-butylphenyl)-N,N'-bis-(2-ethyl-6-methylphenyl)-[p-terphenyl]-4,4"-diamine, N,N'-bis(4-butylphenyl)-N,N'-bis-(2,5-dimethylphenyl)-[p-terphenyl]-4,4"-diamine, N,N'-diphenyl-N,N'-bis(3-chlorophenyl)-[p-terphenyl]-4,4"-diamine molecules, and wherein the hole

transport resinous binder is selected from the group consisting of polycarbonates and polystyrene; an imaging member wherein the photogenerating layer contains a metal free phthalocyanine; a photoconductor wherein the photogenerating layer contains an alkoxygallium phthalocyanine; photoconductive imaging members comprised of a supporting substrate, a photogenerating layer, a hole transport layer, and in embodiments wherein a plurality of charge transport layers are selected, such as for example, from two to about ten, and more specifically two, may be selected; and a photoconductive imaging member comprised of an optional supporting substrate, a photogenerating layer, and a first, second, and third charge transport layer.

The following Examples are being submitted to illustrate embodiments of the present disclosure.

#### Comparative Example 1

A dispersion of a hole blocking layer was prepared by milling 18 grams of  $\text{TiO}_2$  (MT-150W, manufactured by Tayca Co., Japan), 24 grams of a phenolic resin (VARCUM® 29159, OxyChem, Co.) at a solid weight ratio of about 60 to about 40 in a solvent of about 50 to about 50 in weight of xylene and 1-butanol, and a total solid content of about 52 percent in an Attritor mill with about 0.4 to about 0.6 millimeter size  $\text{ZrO}_2$  beads for 6.5 hours, and then filtering with a 20  $\mu\text{m}$  Nylon filter. To the resulting dispersion was then added methyl isobutyl ketone in a solvent mixture of xylene, 1-butanol at a weight ratio of 47.5:47.5:5 (xylene:butanol:ketone). A 30 millimeter aluminum drum substrate was coated using known coating techniques with the above-formed dispersion. After drying a hole blocking layer of  $\text{TiO}_2$  in the phenolic resin ( $\text{TiO}_2$ /phenolic resin=60/40) about 10 microns in thickness were obtained.

A photogenerating layer comprising chlorogallium phthalocyanine (Type B) was disposed on the above hole blocking layer or undercoat layer at a thickness of about 0.2  $\mu\text{m}$ . The photogenerating layer coating dispersion was prepared as follows. 2.7 Grams of chlorogallium phthalocyanine (Cl-GaPc) Type B pigment were mixed with 2.3 grams of polymeric binder (carboxyl-modified vinyl copolymer, VMCH, Dow Chemical Company), 15 grams of n-butyl acetate, and 30 grams of xylene. The mixture was milled in an Attritor mill with about 200 grams of 1 millimeter Hi-Bea borosilicate glass beads for about 3 hours. The dispersion was filtered through a 20  $\mu\text{m}$  Nylon cloth filter, and the solid content of the dispersion was diluted to about 6 weight percent.

Subsequently, a 32 micron charge transport layer was coated on top of the photogenerating layer from a dispersion prepared from N,N'-diphenyl-N,N'-bis(3-methylphenyl)-1,1'-biphenyl-4,4'-diamine (5.38 grams), a film forming polymer binder PCZ 400 [poly(4,4'-dihydroxy-diphenyl-1-1-cyclohexane,  $M_w=40,000$ )], available from Mitsubishi Gas Chemical Company, Ltd. (7.13 grams), and PTFE POLY-FLONTM L-2 microparticle (1 gram) available from Daikin Industries dissolved/dispersed in a solvent mixture of 20 grams of tetrahydrofuran (THF), and 6.7 grams of toluene via a CAVIPROT™ 300 nanomizer (Five Star Technology, Cleveland, Ohio). The charge transport layer was dried at about 120° C. for about 40 minutes.

#### Comparative Example 2

There was prepared a photoconductor with a biaxially oriented polyethylene naphthalate substrate (KALEDEX™ 2000) having a thickness of 3.5 mils, and thereover, a 0.02 micron thick titanium layer was coated on the biaxially ori-

ented polyethylene naphthalate substrate (KALEDEX™ 2000). Subsequently, there was applied thereon, with a gravure applicator or an extrusion coater, a hole blocking layer solution containing 50 grams of 3-aminopropyl triethoxysilane (γ-APS), 41.2 grams of water, 15 grams of acetic acid, 684.8 grams of denatured alcohol, and 200 grams of heptane. This layer was then dried for about 1 minute at 120° C. in a forced air dryer. The resulting hole blocking layer had a dry thickness of 500 Angstroms. An adhesive layer was then deposited by applying a wet coating over the blocking layer, using a gravure applicator or an extrusion coater, and which adhesive contained 0.2 percent by weight based on the total weight of the solution of the copolyester adhesive (ARDEL D100™ available from Toyota Hsutsu Inc.) in a 60:30:10 volume ratio mixture of tetrahydrofuran/monochlorobenzene/methylene chloride. The adhesive layer was then dried for about 1 minute at 120° C. in the forced air dryer of the coater. The resulting adhesive layer had a dry thickness of 200 Angstroms.

A photogenerating layer dispersion was prepared by introducing 0.45 gram of the known polycarbonate IUPILON 200™ (PCZ-200) weight average molecular weight of 20,000, available from Mitsubishi Gas Chemical Corporation, and 50 milliliters of tetrahydrofuran into a 4 ounce glass bottle. To this solution were added 2.4 grams of hydroxygallium phthalocyanine (Type V) and 300 grams of 1/8 inch (3.2 millimeters) diameter stainless steel shot. This mixture was then placed on a ball mill for 8 hours. Subsequently, 2.25 grams of PCZ-200 were dissolved in 46.1 grams of tetrahydrofuran, and added to the hydroxygallium phthalocyanine dispersion. This slurry was then placed on a shaker for 10 minutes. The resulting dispersion was, thereafter, applied to the above adhesive interface with a Bird applicator to form a photogenerating layer having a wet thickness of 0.25 mil. A strip about 10 millimeters wide along one edge of the substrate web bearing the blocking layer and the adhesive layer was deliberately left uncoated by any of the photogenerating layer material to facilitate adequate electrical contact by the ground strip layer of that was applied later. The photogenerating layer was dried at 120° C. for 1 minute in a forced air oven to from a dry photogenerating layer having a thickness of 0.4 micron.

The resulting photoconductor web was then coated with a dual charge transport layer. The first charge transport layer was prepared by introducing into an amber glass bottle in a weight ratio of 50/50, N,N'-bis(methylphenyl)-1,1-biphenyl-4,4'-diamine (TBD) and poly(4,4'-isopropylidene diphenyl) carbonate, a known bisphenol A polycarbonate having a  $M_w$  molecular weight average of about 120,000, commercially available from Farbenfabriken Bayer A.G. as MAKROLON® 5705. The resulting mixture was then dissolved in methylene chloride to form a solution containing 15.6 percent by weight solids. This solution was applied on the photogenerating layer to form the charge transport layer coating that upon drying (120° C. for 1 minute) had a thickness of 16.5 microns. During this coating process, the humidity was equal to or less than 30 percent, for example 25 percent.

The above first pass charge transport layer (CTL) was then overcoated with a second top charge transport layer in a second pass. The charge transport layer solution of the top layer was prepared introducing into an amber glass bottle in a weight ratio of 35/65, N,N'-bis(methylphenyl)-1,1-biphenyl-4,4'-diamine (TBD) and poly(4,4'-isopropylidene diphenyl) carbonate, a known bisphenol A polycarbonate having a  $M_w$  molecular weight average of about 120,000, commercially available from Farbenfabriken Bayer A.G. as MAKROLON® 5705. The resulting mixture was then dissolved in

25

methylene chloride to form a solution containing 15.6 percent by weight solids. This solution was applied, using a 2 mil Bird bar, on the bottom layer of the charge transport layer to form a coating that upon drying (120° C. for 1 minute) had a thickness of 16.5 microns. During this coating process the humidity was equal to or less than 15 percent. The total two-layer CTL thickness was 33 microns.

#### Example I

A photoconductor was prepared by repeating the process of Comparative Example 1 except that there was included in the charge transport layer 0.25 weight percent of the additive 2,4-bis(2,4-dimethylphenyl)-6-(2-hydroxy-4-n-octyl-oxophenyl)-1,3,5-triazine (CYASORB® UV-1164 obtained from CYTEC). The additive was added to the prepared charge transport layer dispersion prior to the coating thereof on the photogenerating layer.

#### Example II

A photoconductor is prepared by repeating the process of Example I except that there is included in the charge transport layer 1 weight percent of the additive a polymer of morpholine-2,4,6-trichloro-1,3,5-triazine, 1,6-hexanediamine, and N,N'-bis(2,2,6,6-tetramethyl-4-piperidinyl)-(CYASORB® UV-3529 obtained from CYTEC,  $M_w \sim 1,700$ ,  $T_g \sim 88^\circ C$ ).

#### Example III

A photoconductor is prepared by repeating the process of Example I except that there is included in the charge transport layer 5 weight percent of the additive poly[(6-morpholino-s-triazine-2,4-diy)[2,2,6,6-tetramethyl-4-piperidyl] imino]-hexamethylene[(2,2,6,6-tetramethyl-4-piperidyl) imino]] (CYASORB® UV-3346 obtained from CYTEC,  $M_w \sim 1,600$ ).

#### Example IV

A photoconductor is prepared by repeating the process of Comparative Example 2 except that there is included in the first charge transport layer 0.5 percent by weight of the additive 2,4-bis(2,4-dimethylphenyl)-6-(2-hydroxy-4-n-octyl-oxophenyl)-1,3,5-triazine (CYASORB® UV-1164 obtained from CYTEC), and the charge transport layer solution components are allowed to mix for 12 hours before coating.

#### Example V

A photoconductor is prepared by repeating the process of Example IV except that there is included in the first charge transport layer 15 weight percent of the additive 2,4,6-tris[phenyl(1-naphthanyl)amino]-1,3,5-triazine.

#### Example VI

A photoconductor is prepared by repeating the process of Example IV except that there is included in the first charge transport layer 10 weight percent of the additive 2,4,6-tris{4-[di(2-pyridyl)amino]phenyl}-1,3,5-triazine.

#### Electrical Property Testing

The above prepared two photoconductors of Comparative Example 1 and Example I were tested in a scanner set to obtain photoinduced discharge cycles, sequenced at one charge-erase cycle followed by one charge-expose-erase

26

cycle, wherein the light intensity was incrementally increased with cycling to produce a series of photoinduced discharge characteristic curves from which the photosensitivity and surface potentials at various exposure intensities were measured. Additional electrical characteristics were obtained by a series of charge-erase cycles with incrementing surface potential to generate several voltages versus charge density curves. The scanner was equipped with a scorotron set to a constant voltage charging at various surface potentials. The 10 photoconductor devices were tested at surface potentials of 700 volts with the exposure light intensity incrementally increased by means of regulating a series of neutral density filters; and the exposure light source was a 780 nanometer light emitting diode. The xerographic simulation was completed in an environmentally controlled light tight chamber at ambient conditions (40 percent relative humidity and 22° C.).

Almost identical PIDC curves were obtained, thus the incorporation of the additive into the charge transport layer did not adversely affect the electrical properties of the photoreceptors.

#### Light Shock Reduction

An in-house light shock test was performed for the above-prepared photoconductor devices (Comparative Example 1 and Example I). The top half of (50 percent) of each of the above-prepared photoconductors was exposed under office light for 60 minutes, and the PIDCs were measured immediately after light exposure. As comparison, the bottom half of the photoconductor was shielded by black paper during the above light exposure, and the PIDCs of the bottom halves were also measured. The light shock results are summarized in Table 1.

TABLE 1

|                       | V(2.65 ergs/cm <sup>2</sup> )<br>of the Shielded<br>Bottom Half (V) | V(2.65 ergs/cm <sup>2</sup> )<br>of the Exposed<br>Top Half (V) |
|-----------------------|---------------------------------------------------------------------|-----------------------------------------------------------------|
| Comparative Example 1 | 279                                                                 | 239                                                             |
| Example I             | 278                                                                 | 259                                                             |

V(2.65 ergs/cm<sup>2</sup>) is the surface potential of the photoconductors when the exposure was 2.65 ergs/cm<sup>2</sup>, and this potential was used to characterize the photoconductors. When the drum devices were exposed from a white light, V(2.65 ergs/cm<sup>2</sup>) was significantly reduced immediately after exposure.

The photoconductor of Example I exhibited a 19V decrease in V(2.65 ergs/cm<sup>2</sup>), whereas the controlled photoconductor of Comparative Example 1 exhibited a 40V decrease in V(2.65 ergs/cm<sup>2</sup>) immediately after office light exposure, which indicated that the Example I photoconductor was more light shock resistant as illustrated by less drop in V(2.65 ergs/cm<sup>2</sup>).

Thus, incorporation of the triazine in the charge transport layer improved light shock resistance with a V(2.65 ergs/cm<sup>2</sup>) drop of about half of that of the controlled photoconductor without the triazine in the charge transport layer.

For an ideal photoconductor, V(2.65 ergs/cm<sup>2</sup>) should 60 remain unchanged whether the photoconductor is exposed to light or not.

Light shock, such as with the photoconductor of Comparative Example 1, causes dark bands to form on xerographic prints when the photoconductors are exposed to light at t=0. The light shock resistant Example I photoconductor did not xerographically print dark bands even when the photoconductor was exposed to light.

The claims, as originally presented and as they may be amended, encompass variations, alternatives, modifications, improvements, equivalents, and substantial equivalents of the embodiments and teachings disclosed herein, including those that are presently unforeseen or unappreciated, and that, for example, may arise from applicants/patentees and others. Unless specifically recited in a claim, steps or components of claims should not be implied or imported from the specification or any other claims as to any particular order, number, position, size, shape, angle, color, or material.

What is claimed is:

1. A photoconductor comprising a supporting substrate, a photogenerating layer, and a first and a second charge transport layer wherein the first charge transport layer is in contact with said photogenerating layer and said first charge transport layer is comprised of a charge transport component and a triazine of poly[(6-morpholino-s-triazine-2,4-diyl)[2,2,6,6-tetramethyl-4-piperidyl]imino]-hexamethylene[(2,2,6,6-tetramethyl-4-piperidyl) imino]], and wherein said charge transport component is comprised of at least one of aryl amine molecules



wherein X is selected from the group consisting of at least one of alkyl, alkoxy, aryl, and halogen.

2. A photoconductor in accordance with claim 1 wherein said triazine is present in an amount of from about 0.01 to about 30 weight percent.

3. A photoconductor in accordance with claim 1 wherein triazine is present in an amount of from about 0.05 to about 10 weight percent.

4. A photoconductor in accordance with claim 1 wherein said triazine is present in an amount of from about 0.1 to about 5 weight percent.

5. A photoconductor in accordance with claim 1 wherein said alkyl and said alkoxy each contains from about 1 to about 12 carbon atoms, and said aryl contains from about 6 to about 36 carbon atoms.

6. A photoconductor in accordance with claim 1 wherein said aryl amine is N,N'-diphenyl-N,N-bis(3-methylphenyl)-1,1'-biphenyl-4,4'-diamine.

7. A photoconductor in accordance with claim 1 further including in at least one of said first and said second charge transport layers an antioxidant comprised of at least one of a hindered phenolic and a hindered amine.

8. A photoconductor in accordance with claim 1 wherein said photogenerating layer is comprised of at least one photogenerating pigment.

9. A photoconductor in accordance with claim 8 wherein said photogenerating pigment is comprised of at least one of a metal phthalocyanine, a metal free phthalocyanine, and a perylene.

10. A photoconductor in accordance with claim 8 wherein said photogenerating pigment is comprised of a titanyl phthalocyanine.

11. A photoconductor in accordance with claim 8 wherein said photogenerating pigment is comprised of a hydroxygallium phthalocyanine.

12. A photoconductor in accordance with claim 8 wherein said photogenerating pigment is comprised of a chlorogallium phthalocyanine.

13. A photoconductor in accordance with claim 8 wherein said photogenerating pigment is comprised of a bis(benzimidazo)perylene.

14. A photoconductor in accordance with claim 1 further including a hole blocking layer, and an adhesive layer.

15. A photoconductor in accordance with claim 1 wherein said substrate is a flexible web.

16. A photoconductor in accordance with claim 1 wherein the substrate is comprised of a conductive material.

17. A photoconductor comprised in sequence of a supporting substrate, a photogenerating layer comprised of at least one photogenerating pigment, and a charge transport layer of a first pass charge transport layer and a second pass charge transport layer over said first pass charge transport layer, and wherein said first pass charge transport layer is in contact with said photogenerating layer and which first pass charge transport layer contains a triazine selected from the group consisting of a polymer containing morpholine-2,4,6-trichloro-1,3,5-triazine, and poly[(6-morpholino-s-triazine-2,4-diyl)[2,2,6,6-tetramethyl-4-piperidyl] imino]-hexamethylene[(2,2,6,6-tetramethyl-4-piperidyl) imino]] present in said first pass charge transport layer in an amount of from about 0.05 to about 10 weight percent.

18. A photoconductor in accordance with claim 17 wherein said triazine is present in an amount of from about 0.1 to about 7 weight percent.

19. A photoconductor in accordance with claim 17 wherein the charge transport layer is comprised of hole transport molecules and a resin binder, said photogenerating pigment is a titanyl phthalocyanine prepared by dissolving a Type I titanyl phthalocyanine in a solution comprising a trihaloacetic acid and an alkylene halide; adding said mixture comprising the dissolved Type I titanyl phthalocyanine to a solution comprising an alcohol and an alkylene halide thereby precipitating a Type Y titanyl phthalocyanine; and treating said Type Y titanyl phthalocyanine with a monohalobenzene, and wherein said photoconductor contains a supporting substrate.

20. A photoconductor in accordance with claim 19 wherein said solution comprising an alcohol and an alkylene halide has an alcohol to alkylene halide ratio of from about 1/4 (v/v) to about 4/1 (v/v), and said titanyl phthalocyanine is Type V titanyl phthalocyanine, and wherein the resulting Type V titanyl phthalocyanine has an X-ray diffraction pattern having characteristic diffraction peaks at a Bragg angle  $2\Theta \pm 0.2^\circ$  at about  $9.0^\circ$ ,  $9.6^\circ$ ,  $24.0^\circ$ , and  $27.2^\circ$ .